

July 18, 1944.

B. W. ROWLAND ET AL

2,353,852

METHOD OF DETERMINING THE RECEPCEPTIVITY OF SHEET

MATERIALS TO COATINGS, INKS, AND THE LIKE

Filed March 7, 1942

2 Sheets-Sheet 1



Fig. 1



July 18, 1944.

B. W. ROWLAND ET AL.

2,353,852

METHOD OF DETERMINING THE RECEPITIVITY OF SHEET MATERIALS TO COATINGS, INKS, AND THE LIKE

TO COATINGS, INKS, AND  
FILED MARCH 7, 1942

2 Sheets-Sheet 2



Inventors:  
Ben W. Rowland,  
Douglas Frommutter  
and Johannes A. Van den Akker,  
By Soans, Pond & Anderson  
Attorneys.

## UNITED STATES PATENT OFFICE

2,353,852

METHOD OF DETERMINING THE RECEP-  
TIVITY OF SHEET MATERIALS TO COATINGS,  
INKS, AND THE LIKEBen W. Rowland, Douglas Fronmuller, and Jo-  
hannes A. Van den Akker, Appleton, Wis., as-  
signors to The Institute of Paper Chemistry, a  
corporation of Wisconsin

Application March 7, 1942, Serial No. 433,822

3 Claims. (Cl. 73—51)

The present invention relates to a testing method for determining and evaluating various surface characteristics of sheet materials, and particularly of paper.

In the past, considerable difficulty has been experienced in determining the receptivity of paper and similar products to coating materials, inks, and the like. Prior to the investigation resulting in the present invention it was generally believed that unsatisfactory coatings resulted from some inherent defect in the raw stock from which the sheet was made. Testing procedures were developed on this theory, but these proved generally unsatisfactory and the only true evaluation of the receptivity characteristics that could be reached involved applying the actual coating material to the sheet.

In our investigations, directed toward the overcoming of the deficiencies of the prior art testing procedures, we have discovered that the receptivity of paper and like sheet materials for coatings, inks, etc., is related to the surface characteristics of such materials, and as will herein-after appear, we have provided apparatus for accurately evaluating such characteristics to the end that the receptivity of any particular sheet to coatings, inks, etc., may be determined, even while the sheet is being manufactured. The testing apparatus of our invention is substantially automatic in operation, and it performs the testing operation with substantially no rubbing or mechanical working of the surface which is to be tested, an important feature in view of the relationship which we have found to exist between receptivity to coatings and surface characteristics. Moreover, the apparatus of our invention is simple and relatively inexpensive; it is rapid and easy to operate; and the results are substantially unaffected by the technique of operation.

One embodiment of our invention, particularly designed for evaluating the receptivity of paper to coating materials and inks, is illustrated in the accompanying drawings and more fully described in the following description. In the drawings:

Fig. 1 is a perspective view of the complete apparatus;

Fig. 2 is an enlarged sectional view on the general line 2—2 of Fig. 1;

Fig. 3 is a sectional view on line 3—3 of Fig. 2;

Fig. 4 is a sectional view on the line 4—4 of Fig. 3 and shows a bottom plan view of one of the plate elements comprising the doctor or scraper blade of the structure shown in Figs. 1 and 3;

Fig. 5 is a top plan view of the other element forming the doctor blade;

Fig. 6 is an enlarged sectional view showing the operation of the doctor blade; and

Fig. 7 is an enlarged sectional view of the fluid trap forming a part of the apparatus.

Reduced to its basic elements the testing apparatus of the present invention comprises means, including a resilient platen, for holding the sheet of paper or other material to be tested substantially flat, and means including a vacuum doctor or scraper mechanism for advancing a quantity of a suitable testing fluid across the surface of the sheet and for immediately thereafter removing any excess from the surface of such sheet. In the particular embodiment illustrated in the drawings, this latter means includes an electric motor or other apparatus for moving the doctor mechanism across the sheet being tested at a uniform, relatively high speed.

More specifically, the apparatus includes a suitable base 11 of wood or metal provided with a pair of rigid uprights 13 which serve as the support means for a pair of spaced, parallel guide rails 15. The operating and support means for the vacuum doctor blade mechanism comprises a relatively heavy, metallic plate 17 having a pair of spaced, parallel grooves 19 cut therein, for slidably engaging the guide rails 15. The platen support for the sample includes a sheet of plate glass 21 of suitable dimensions which is positioned on the main base 11 in the area beneath the guide rails 15 and a spring operated, press clip 23 for holding the sample.

To provide a resilient support for the sample, a flat pad or cushion 25 of uniform thickness is disposed on top of the glass plate 21. The resilient pad 25 may comprise a plurality of superposed sheets of paper, or a sheet of rubber or other material, and should be located between the sample and the plate 21 during the operation of the apparatus. In one particularly satisfactory embodiment of the invention the glass plate 21 has a width of about 5 inches and a length of approximately 15 inches. The resilient pad 25 in this embodiment is about one-eighth inch thick and comprises approximately twenty sheets of a relatively hard paper.

The supporting plate 17 for the vacuum doctor mechanism is moved longitudinally of the apparatus by means of an electric motor 27, a belt 29 which extends through suitable openings 31 in the uprights 13, a fixed pulley 33, and a motor pulley 34 about which the belt is wrapped once around. In the interest of smooth, quick starting, a spring 36 is preferably interposed in the belt circuit.

A start and stop switch 38 for the motor 27 is

supported on the right hand upright 13 and is connected into the electrical circuit for the motor in conventional manner. In the particular apparatus shown in the drawings, the plate 17 and the doctor blade mechanism which is supported thereon are returned to the initial operating position by hand. It will be understood, however, that a mechanical return can be used if desired, as for example, by providing a reversing motor. The motor switch 38 is so arranged that it automatically shuts off the motor 27 when the supporting plate 17 approaches the right hand end of the apparatus during the operation of the machine.

In the illustrated device, the vacuum doctor blade mechanism includes a two element doctor blade 35 which is hingedly supported on the main plate 17 by means of a support arm 37 and a U-shaped spring hinge 39. The spring hinge 39 includes adjustable tension springs 41 which serve to bias the doctor blade in the direction of the sample support means. The support arm 37 which provides the mechanical connection between the spring hinge 39 and the two element doctor blade 35 is integrally attached at one end to the lower elements 43 of the doctor blade and is threaded at the other end for engagement with a suitable threaded block 45 integrally attached to the lower element of the hinge 39. It will be apparent that the angle of the doctor blade relative to the plane of the sample support can be readily adjusted by screwing the supporting arm 37 in or out of the threaded block element 45.

The two elements of the doctor blade 35 are particularly shown in Figs. 4, 5, and 6. The lower element 43 has a beveled under surface 47 which is adapted to rest on the surface of the sample during the operation of the machine. The angle of this bevel should be such that when the surface 47 rests flat on the sample the angle between the doctor blade and the plane of the sample, the angle A of Fig. 6, will be about 30 to 35 degrees. The lower doctor blade element 43 is provided with two upstanding side portions 49 for receiving and guiding the upper element 51. The upper doctor blade element 51, is shown in bottom plan view in Fig. 4 and comprises a metallic plate which is cut away on its under surface as illustrated at 53 in Figs. 4 and 6. When the two elements 43 and 51 are assembled, this cut away portion 53 provides an outwardly flaring, vacuum chamber 55 which extends along substantially the entire width of the doctor blade. The upper element 51 is adjustably fastened to the lower element 43 by means of suitable screws 57, which engage threaded openings 59 in the lower element and which pass through slotted openings 61 in the upper element. The lower surfaces of the end edge portions 63 of the upper element 51 are beveled to the same angle as the surface 47 of the lower element 43 in order that the doctor blade may rest flat against the sample being tested. The engaging surfaces of the two elements 47 and 51 are preferably ground to a very close fit and for best results it is highly desirable that the bevel surfaces 47 and 63 which contact the sample shall be perfectly flat. In one particularly satisfactory embodiment of the invention the doctor blade had a total width of approximately 7.0 cm. and a width at the beveled portion of about .7 cm. Approximately this ratio is believed desirable. Subatmospheric pressure is maintained within the vacuum chamber 55 during the operation of the apparatus by the use of any suitable mechanism. In the particular ap-

paratus illustrated in the drawings, this reduced pressure is provided by means of a Venturi aspirator 65, which is connected to a suitable fluid source through a valve 67 as illustrated in Fig. 1. The aspirator 65 is connected to the vacuum chamber 55 through suitable flexible tubing 69 and a trap 71 which is supported directly on the doctor blade structure 35, the trap being connected to the chamber by a short piece of flexible tubing 73 and a metallic tube 75 which extends through the upper doctor blade element 51. To facilitate control and adjustment of the apparatus a vacuum gauge 77 is provided. The gauge is preferably connected into the tubing 69, and under normal operating conditions, it will be found advisable to adjust the vacuum within the chamber 55 to about 15 to 20 centimeters of mercury below atmospheric.

A substantial amount of liquid is drawn into the vacuum chamber 55 during the operation of the apparatus, and the trap 71 is particularly useful in maintaining even pressure in this chamber. Preferably, the trap 71 should be of glass to permit visual examination, and it should be so designed that it includes spaced entrance and exit passageways 79 and 81, as illustrated in Fig. 7. It is desirable that the level of the exit passageway 81 shall be below the level of the entrance passageway 79 to minimize sudden changes in pressure. To facilitate cleaning, one end of the trap may be left open and sealed with a rubber cap 83. In some instances, it may be desirable to provide vanes or baffles within the vacuum chamber as indicated by the dotted lines 85 in Fig. 4, for the purpose of equalizing fluid flow therein. Generally, however, these vanes are unnecessary.

The preferred testing procedure includes the following steps: A sample of the paper or other material to be tested is fastened in place on the sample supporting pad 25 by the spring clip 23, as illustrated at 81. The sample 81 should have a width greater than the width of the doctor blade 35 and a length at least equal to the length of the travel of the doctor blade. By virtue of the spring hinge connection between the doctor blade 35 and the support and operating means therefor, the doctor blade can be readily lifted to permit the sample to be put into place.

Before starting the test, the doctor blade 35 and its operating mechanism are moved to the extreme left hand position, as shown in Fig. 1. Also before starting the test, the aspirator 65 or other vacuum producing apparatus must be turned on, as by operation of the valve 67, and the pressure within the vacuum chamber 55 of the doctor blade structure 35 adjusted to the desired value. As stated previously in making tests to determine the receptivity of paper to coating materials, best results are obtained with a pressure in the vacuum chamber of about 15 to 20 centimeters of mercury below atmospheric. With the apparatus in the starting position, as described, a quantity of the testing fluid is applied, by means of a medicine dropper or otherwise, to form a pool of liquid 89 (Fig. 6) directly ahead of the doctor blade 35, as illustrated in Fig. 6. Thereupon, the motor switch 38 is operated to effect the energization of the motor 27 which moves the doctor blade mechanism, at relatively high speed, from the position illustrated in full in Fig. 3 to the position illustrated in dotted lines in that figure. This movement of the doctor blade mechanism, in combination with the doctoring action resulting from the vacuum which is maintained within the chamber 55 causes a

very thin coating of the testing material to be spread over the surface of the sample being tested in a very short interval of time. Speeds of the order of about 20 to 30 inches per second have been used with very good results. This coating will form patterns which can be readily evaluated as a measure of the receptivity of the sheet to coating materials. If the pattern is uniform and continuous, the material has a high degree of receptivity for the coating materials, and particularly for those coating materials which comprise a mixture of an adhesive, such as casein or starch, and a pigment, such as clay, satin white or some other of the known coating pigments. If the pattern is discontinuous and contains fish eyes or other irregularities, difficulty in coating may be expected, the amount of difficulty being directly proportional to the amount of discontinuance in the pattern. Comparative, reference standards may be set up for any particular test or series of tests. By virtue of the fact that the liquid testing material is applied ahead of the doctor blade, it is probable that lubrication of the doctor blade element takes place during its movement over the surface of the sample to be tested. This action, in combination with the relatively large bearing surface of the doctor blade element and the rather moderate pressures used, appears to effectively prevent any mechanical working of the surface of the sample, which might tend to give erroneous indications of the receptivity of the surface to coating. In the described embodiment, pressures are used of the order of 100 grams total across the entire contact area of the doctor blade, and while some variation in this pressure may be permissible, best results appear to be obtained with approximately this pressure. The period of time required to make tests by use of the apparatus of the present invention is so short that close control of the actual manufacture operation is made possible in the case of paper and like materials.

As stated previously, the test may be used not only for determining the receptivity of sheet material to coating, but also the receptivity of previously coated sheets to ink, or to other liquids. In these instances, use of some different type of testing fluid may be indicated. For determining coatability, we prefer to use an aqueous, colored medium, preferably a colloid, although in some instances ordinary suspensions have proven satisfactory. For other tests, other testing liquids of greater or less viscosity may be desirable and the term "fluid testing material" as used herein is intended for all such materials.

It will be apparent that various other devices embodying the principles disclosed in the foregoing may be developed by those skilled in the art. Accordingly, it is desired that the accompanying claims shall be given the broadest reasonable construction consistent with the language appearing therein and the prior art.

We claim:

1. The method of determining the receptivity of sheet material to coatings, inks, and the like which consists in supporting a sample of the material to be tested on a suitable, resilient surface, applying a substantial quantity of a fluid testing material to a restricted area of the sample, spreading said fluid testing material over the sample at relatively high speed, while immediately doctoring off as much of the spread testing material as is possible from the surface of the sample by use of a suction current, thereby effecting the very rapid application of a very thin coating of the testing material to the surface of the sample, the said application of testing material being carried out without substantial mechanical working of the surface of the sample, and finally evaluating the resulting pattern by comparison with known standards.
- 10 2. The method of determining the receptivity of sheet material to coatings, inks, and the like which consists in supporting a sample of the material to be tested on a suitable, resilient surface, applying a substantial quantity of a fluid testing material to a restricted area of the sample, spreading said fluid testing material over the sample at a speed which is of the order of about 20 to 30 inches per second, while immediately doctoring off as much of the spread testing material as is possible from the surface of the sample by the use of a suction current of the order of about 15 to 20 centimeters of mercury, thereby effecting the very rapid application of a very thin coating of the testing material to the surface of the sample, the said application of testing material being carried out without substantial mechanical working of the sample, and finally evaluating the resultant pattern by comparison with known standards.
- 20 3. The method of determining the receptivity of sheet material to coatings, inks, and the like which consists in applying a substantial quantity of a fluid testing material to a restricted area of the sample, spreading said fluid testing material over the sample at relatively high speed, while immediately doctoring off as much of the spread testing material as is possible from the surface of the sample by use of a suction current, thereby effecting the very rapid application of a very thin coating of the testing material to the surface of the sample, the said application of testing material being carried out without substantial mechanical working of the surface of the sample, and finally evaluating the resultant pattern by comparison with known standards.
- 25 4. The method of determining the receptivity of sheet material to coatings, inks, and the like which consists in applying a substantial quantity of a fluid testing material to a restricted area of the sample, spreading said fluid testing material over the sample at a speed which is of the order of about 20 to 30 inches per second, while immediately doctoring off as much of the spread testing material as is possible from the surface of the sample by the use of a suction current of the order of about 15 to 20 centimeters of mercury, thereby effecting the very rapid application of a very thin coating of the testing material to the surface of the sample, the said application of testing material being carried out without substantial mechanical working of the sample, and finally evaluating the resultant pattern by comparison with known standards.
- 30 5. The method of determining the receptivity of sheet material to coatings, inks, and the like which consists in applying a substantial quantity of a fluid testing material to a restricted area of the sample, spreading said fluid testing material over the sample at a speed which is of the order of about 20 to 30 inches per second, while immediately doctoring off as much of the spread testing material as is possible from the surface of the sample by the use of a suction current of the order of about 15 to 20 centimeters of mercury, thereby effecting the very rapid application of a very thin coating of the testing material to the surface of the sample, the said application of testing material being carried out without substantial mechanical working of the sample, and finally evaluating the resultant pattern by comparison with known standards.
- 35 6. The method of determining the receptivity of sheet material to coatings, inks, and the like which consists in applying a substantial quantity of a fluid testing material to a restricted area of the sample, spreading said fluid testing material over the sample at a speed which is of the order of about 20 to 30 inches per second, while immediately doctoring off as much of the spread testing material as is possible from the surface of the sample by the use of a suction current of the order of about 15 to 20 centimeters of mercury, thereby effecting the very rapid application of a very thin coating of the testing material to the surface of the sample, the said application of testing material being carried out without substantial mechanical working of the sample, and finally evaluating the resultant pattern by comparison with known standards.
- 40 7. The method of determining the receptivity of sheet material to coatings, inks, and the like which consists in applying a substantial quantity of a fluid testing material to a restricted area of the sample, spreading said fluid testing material over the sample at a speed which is of the order of about 20 to 30 inches per second, while immediately doctoring off as much of the spread testing material as is possible from the surface of the sample by the use of a suction current of the order of about 15 to 20 centimeters of mercury, thereby effecting the very rapid application of a very thin coating of the testing material to the surface of the sample, the said application of testing material being carried out without substantial mechanical working of the sample, and finally evaluating the resultant pattern by comparison with known standards.
- 45 8. The method of determining the receptivity of sheet material to coatings, inks, and the like which consists in applying a substantial quantity of a fluid testing material to a restricted area of the sample, spreading said fluid testing material over the sample at a speed which is of the order of about 20 to 30 inches per second, while immediately doctoring off as much of the spread testing material as is possible from the surface of the sample by the use of a suction current of the order of about 15 to 20 centimeters of mercury, thereby effecting the very rapid application of a very thin coating of the testing material to the surface of the sample, the said application of testing material being carried out without substantial mechanical working of the sample, and finally evaluating the resultant pattern by comparison with known standards.
- 50 9. The method of determining the receptivity of sheet material to coatings, inks, and the like which consists in applying a substantial quantity of a fluid testing material to a restricted area of the sample, spreading said fluid testing material over the sample at a speed which is of the order of about 20 to 30 inches per second, while immediately doctoring off as much of the spread testing material as is possible from the surface of the sample by the use of a suction current of the order of about 15 to 20 centimeters of mercury, thereby effecting the very rapid application of a very thin coating of the testing material to the surface of the sample, the said application of testing material being carried out without substantial mechanical working of the sample, and finally evaluating the resultant pattern by comparison with known standards.
- 55 10. The method of determining the receptivity of sheet material to coatings, inks, and the like which consists in applying a substantial quantity of a fluid testing material to a restricted area of the sample, spreading said fluid testing material over the sample at a speed which is of the order of about 20 to 30 inches per second, while immediately doctoring off as much of the spread testing material as is possible from the surface of the sample by the use of a suction current of the order of about 15 to 20 centimeters of mercury, thereby effecting the very rapid application of a very thin coating of the testing material to the surface of the sample, the said application of testing material being carried out without substantial mechanical working of the sample, and finally evaluating the resultant pattern by comparison with known standards.

BEN W. ROWLAND.  
DOUGLAS FRONMULLER.  
JOHANNES A. VAN DEN AKKER.